

# UNITED STATES PATENT OFFICE.

PHILIP CAREY, OF CINCINNATI, OHIO.

## ROOFING MATERIAL.

SPECIFICATION forming part of Letters Patent No. 402,559, dated May 7, 1889.

Application filed December 22, 1888. Serial No. 294,378. (No specimens.)

*To all whom it may concern:*

Be it known that I, PHILIP CAREY, a citizen of the United States, residing at Cincinnati, in the county of Hamilton and State of Ohio, 5 have invented a certain new and useful Improvement in Roofing Material, of which the following is a full, clear, and exact description.

My invention relates to an improvement in roofing material; and it consists of the roofing- 10 felt ordinarily used for that purpose saturated in a mixture consisting of petroleum, lamp-black, and asphaltum, which mixture is used as a substitute for the ordinary coal-tar. Coal-tar, which is generally used, is objection- 15 able for several reasons—among them, its cost; also the fact that after it has been exposed to the weather for some time it becomes brittle and loses its vitality. The heavier petroleum-oils may be rendered practically 20 odorless by distillation. With this distilled oil I mix a sufficient amount of lamp-black to bring it to about the consistency of liquid tar and add a small quantity of asphaltum, rosin, or other similar substance, which produces a 25 stiffening and drying effect. The felt, having been saturated or passed through this compound, is passed between rollers in the usual way, to press in the mixture and remove the surplus, when it may be rolled into rolls for 30 use, or may be put through the machine for uniting several thicknesses and producing a two-ply or three-ply felt. Ordinarily, in the use of oils for this purpose, or a mixture containing oils, there is left upon the surface of 35 the paper a greasy or oily substance, which makes them objectionable to the trade, because with this oily surface the felt is unpleasant to handle, and if it is rolled into rolls the greasy substance is liable to become 40 gummy and make them more or less sticky. To remedy this it is often necessary to use some other process or apply some kind of powder to the surface of the felt. Again, when it is desired to unite several sheets, the 45 greasy surface prevents the perfect union and

leaves them liable to part. The lamp-black used, as described, leaves the surface of the felt dry and free from the objections named. If mixed with the oil, as described, it is so light that there is no tendency to settle at the 50 bottom, as heavier substances are liable to do; but, on the contrary, there is a chemical union between the oil and the lamp-black forming a homogeneous compound. The proportions I use are about one-half or five-tenths of the 55 oil, four-tenths of lamp-black, and one-tenth asphaltum.

I do not limit myself to these proportions exactly, as the amount of lamp-black differs with different oils, my discovery relating 60 especially to the use of lamp-black with oil for the purposes described. This preparation is easily handled and easily applied, is inexpensive, and very much superior in its result to any other compound that I know of. With 65 slight modifications it may be used for a paving compound, the modifications depending upon the climate in which it is to be used, as is well known, the requirement for hot and cold climates varying in all such compounds. 70

Rosin possesses some of the qualities of asphaltum as a drying and stiffening ingredient, and may be used as a substitute for or mixed with the asphaltum. The use of either is 75 simply for the purpose described, and I do not limit myself to any particular substance for that purpose.

Having thus fully described my invention, what I claim, and desire to secure by Letters Patent, is—

A roofing or paving material consisting of the above-described compound of distilled petroleum, lamp-black, and asphaltum, or its equivalent, combined substantially in the proportions and for the purpose described.

PHILIP CAREY.

Witnesses:

ALFRED M. ALLEN,  
GEORGE HEIDMAN.